

## UNITED STATES PATENT OFFICE

GUSTAV ULLMANN, OF VIENNA, AUSTRIA

## BUCKING PROCESS FOR VEGETABLE FIBROUS MATERIAL

No Drawing. Application filed January 24, 1930, Serial No. 423,385, and in Austria January 26, 1929.

Vegetable fibres such as cotton, flax, juts etc. are loaded with a large number of natural impurities, the removal of which is the object of the boiling or bucking process which is frequently carried out for the purification of vegetable fibres in many refining processes and must be carried out in the bleaching process. After boiling there remains principally on the fibre the natural colouring matter, which is then removed in the well known way, usually by treatment with an oxidizing agent, such as chloride of lime, peroxides and the like.

The impurities to be removed by the boiling or bucking process are of the most various kinds. Cotton, for example, which is the principal representative of the vegetable fibres contains principally:

1. Fatty and waxy substances.
2. Pectin substances.
3. Albuminoids.
4. The natural colouring matters.
5. The woody and husk portions.

The different behaviour of the impurities towards the various reagents employed in bucking makes the bucking process very difficult to carry out. The impurities are soluble to a slight extent in water and to a greater extent in alkalies or alkali earths while the fats and waxes can only be removed from the fibre by saponification or by melting them out and emulsifying them. The fats and waxes, in particular, must be removed, because they completely surround the fibres and prevent the access thereto of the other chemicals and solvents.

Scheurer has determined comparatively, in a long series of experiments the velocities of saponification when boiling with all kinds of chemicals, such as caustic and carbonated alkalies, alkali earths and other metallic salts and additions. Just as he gave precedence to  $\text{Ca}(\text{OH})_2$ , which is principally used in practice so, in the explanation of the present invention, the reactions which take place will be described with reference to lime compounds but this is not to be taken as meaning that the scope of the invention is so restricted accordingly. Scheurer's investigations have shown, inter alia, that calcium hydroxide

both when used under ordinary pressure and when under superatmospheric pressure, that is to say, at temperatures up to 100° C. and higher, effects the most rapid saponification of the fatty and waxy substances and carries it out in a much shorter time than comparatively high percentages of caustic alkali or carbonated alkali. A circumstance which must be regarded as a particular advantage of boiling with lime is that the velocity of circulation does not play any important part in the process, that is to say, the chemical process of saponification and the removal of the fatty substances and other impurities is not dependent in the same degree on the quantity of material treated at one time in a boiler as when boiling is carried out with solutions of caustic alkalies or soda.

Boiling with lime alone, however, can never effect an adequate purification of the fibrous material; it must always be followed by boiling with a caustic or a carbonated alkali. Ordinarily after being boiled with lime, the fibrous material is washed, acidified, washed again and then boiled with an alkali. The two boilings together are shorter, that is to say they take up less time than one boiling with alkali alone. At the same time, boiling with lime introduces other advantages. The white of the bleached material obtained thereby is always better, more "bluish"; the thread is smoother, probably owing to the fact that in boiling with lime the lime paste envelopes and protects the threads or the fabric.

Despite these important advantages boiling with lime and alkalies has been more and more displaced by boiling with alkalies alone and the chief reason for this being that the latter method can be carried out in a single operation, whereas after the lime boiling process carried out as above described, two or if the acidification be included, three operations are necessary. When boiling with alkalies various additions to the bucking liquors have been suggested and used in order to assist the emulsification of the impurities and the wetting of the fibrous material, but nothing further will be said of these added substances in this connection. All these sub-

55

60

65

70

75

80

85

90

95

100

stances are, however, merely for the purpose of accelerating the boiling with alkalies and this not only for obvious economical reasons (since prolonged boiling entails increased expense for steam and labour and lessens the yield of the apparatus) but more particularly, because short boiling brings with it the conservation of the fibrous material in an undamaged state, on which the greatest value must be placed. Nevertheless, boiling with alkalies alone has not secured the advantage as regards shortness of time and superior appearances of the material, which is obtained when the fibre is boiled both with lime and with alkalies.

15 Simultaneous treatment of the fibre with lime and alkali compounds has not hitherto been found possible, as the lime soaps which are formed prevent the access of the caustic alkali to the fibre, and carbonated alkalies could not be used owing to their precipitating action on lime water.

20 The present invention enables the high saponifying action of calcium hydroxide to be utilized in the boiling of fibrous material and at the same time, that is to say, in one single operation, it enables the lime soaps which are formed to be brought into solution or converted into a highly dispersed form, so that they can easily be rinsed off from the fibre. This idea can be carried out in various ways. One mode of carrying out the invention consists in boiling vegetable fibres either under increased pressure or at ordinary pressure with a liquor which contains, in addition to a caustic alkali, metallic hydroxide which forms insoluble soaps, e. g.  $\text{Ca}(\text{OH})_2$ ,  $\text{Ba}(\text{OH})_2$ ,  $\text{Sr}(\text{OH})_2$ ,  $\text{AL}_2(\text{OH})_6$ ,  $\text{Fe}_2(\text{OH})_6$  or a salt of such metals and also a substance 25 which passes into a soluble or a high dispersed compound with the metal. Such substances are the well known soluble oil preparations which are insensitive to lime and which are obtained by the sulphonation of 30 castor oil and other oils and subsequently boiling them with alkalies, also sulphonation products of unsaturated fatty acids and resins. Bodies may also be used which are of quite a different chemical nature and are used 35 for avoiding inconveniences which would otherwise be caused by the presence in water of metallic soaps and also as wetting agents for spun fibres. Thus, for instance, the sulphonic acids of polynuclear aromatic hydrocarbons with alkyl side chains and other substances the metallic compounds of which 40 behave in a similar manner may be used.

45 In this process lime soaps are formed very rapidly, even at low temperatures and with a limited circulation of the liquid, because the lime acts much more energetically on the fatty acids and saponifies them more rapidly than caustic alkalies or alkali carbonates. If only lime and an alkali were used the insoluble lime soaps would envelop the fibres

50 and obstruct the alkalies which possess a much higher coefficient of solution and emulsification for the other natural impurities in the fibres and the woody parts and would prevent said alkalies from reaching these impurities. It is only by the addition of the third reagent that the lime soap is either dissolved or brought into a highly dispersed form so that the alkali can penetrate into the fibre and dissolve or emulsify the various 55 impurities contained therein. The process therefore renders it possible to work with lime and an alkali in a single bath without introducing the aforementioned disadvantages and to do this in such a way that each of the reagents is able to develop to the full its best possible solvent, saponifying or emulsifying action.

60 As the process according to this invention permits of carrying out the bucking process in a highly accelerated form and effects a more thorough purification under ordinary pressure than heretofore, it is particularly suitable also for bleaching coloured textiles and continuous bleaching, which is mostly 65 carried out as piece bleaching. For bleaching coloured textiles the present process has the advantage that the fibres are conservated in a better manner by the shortening of the time of boiling and by the avoidance of increased pressure, although a more thorough 70 purification takes place than in the bleaching processes for coloured textiles hitherto employed.

75 In continuous bleaching on the basis of the present process considerable simplification of the apparatus is secured as the work does not have to be carried out under pressure. As is well known the means for continuous bleaching under high pressure are 80 so complicated and difficult to supervise and their work so difficult to control that it has not hitherto been possible, in practice, to introduce this method of working, which would otherwise be very advantageous, while bleaching 85 in open vessels on the continuous process has hitherto not yield any satisfactory results.

90 Another mode of carrying out this invention consists in introducing into the boiling liquor, in addition to a caustic alkali, a metallic compound of those oil preparations or other emulsifying agents which are capable of dissolving the metallic soaps produced from the fats and waxes, or of bringing them 95 into a highly dispersed form. Finally, the invention also extends to the production of the reagents required to carry out this process, that is to say, to the production of metallic compounds of oil preparations, sulphonic acids of polynuclear aromatic hydrocarbons with alkyl side chains and the like, all of which bodies behave in the above mentioned 100 manner towards metallic soaps.

105 The basis of the process described is, doubt- 110

less, the saponifying action of the lime, but it is of no consequence if this be present in a quantity below the stoichiometric in proportion to the particular fats and waxes contained in the fibre, because the caustic alkali and the other substances added have also a saponifying and emulsifying action. As a rule, however, the work is carried out in first instance for reasons of economy with an excess of lime over the approximate actual consumption thereof which latter can be estimated, as the amount of fat and wax contained in cottons of various origins (e. g. East Indian, Egyptian, American and others) is known from the outset just as in the other fibrous materials.

*Examples*

1. In a boiler containing 2000 kg. of cotton material to be boiled out and about 8000 litres of bucking liquor there are used for the boiling out process.

500 g. calcium oxide (CaO) in the form of lime water.

25 30 kg. solid caustic soda (NaOH).

6 kg. of a sulphonated oil containing 60 per cent of fatty acids and insensitive to lime.

After boiling has been carried out for about 4 hours at 100° C. without pressure or after 30 about 2½ hours boiling at a pressure of 2 atm. above atmospheric pressure, the bucking process is complete. The charge is then washed, acidified if necessary washed again and the material, which has also become considerably lighter in colour is treated in the usual way with quite dilute chloride of lime solutions or peroxides and the like and the bleaching process terminated in the usual way. Or the material, which is to be boiled

40 only, may after being boiled, washed and acidified, and then washed once more and dried. A very thorough preliminary bleaching is thus obtained, which frequently makes a further white bleaching quite unnecessary,

45 e. g. for light shades of colour.

2. The material and the liquor are selected as in Example 1. Boiling is carried out with 80 kg. calcium oxide (CaO) and 12 kg. isopropylnaphthylamine sulphonate of sodium 50 or a substance of similar composition and acting in a similar manner. The material is then washed with water, acidified, preferably with hydrochloric acid, washed again and then bleached.

55 3. Material and the liquor as in Example 1. 380 g. of calcium oxide (CaO), 40 kg. of solid caustic soda and 4600 g. of an oil containing 60 per cent of fatty acid and insensitive to lime are taken. The subsequent treatment is as in Example 1.

4. Material and liquor as in Example 1. 35 kg. of solid caustic soda and the barium compound of the dispersing agent are added. The latter is produced as follows:

60 1300 g. of barium hydroxide are stirred

with the corresponding quantity of water and slowly mixed with a solution of 3800 g. of isopropylnaphthylamine sulphonate acid while stirring continuously.

Instead of the barium salt of the said aromatic sulphonate acid the calcium salt of sulphonated unsaturated fatty acids may, for example, be taken. This is prepared as follows:

4750 g. of sulphonated castor oil containing 60 per cent of fatty acid are mixed gradually, whilst being stirred, with a milk of lime prepared from 460 g. of commercial burned lime. The product obtained is concentrated and used in the form of a slip or slurry.

What I claim is:—

1. In a bucking process for vegetable fibrous materials the method consisting in boiling the fibrous material to be treated in a liquor containing caustic alkalies, metallic hydroxides and substances adapted to cause the compounds produced from the natural fats and waxes of the fibrous material during boiling to assume a form in which such compound can easily be washed from the said material.

2. In a bucking process for vegetable fibrous materials, the method consisting in boiling the fibrous material to be treated in a liquor containing caustic alkalies, metallic hydroxides and substances adapted to convert the insoluble compounds which would normally be formed with the natural fats and waxes of the fibrous material into a form such that substantially all the impurities disengaged from the material during boiling can be washed out of the fibres of said material.

3. In a bucking process for vegetable fibrous material, the method of treating the material simultaneously and in one single operation with caustic alkalies and metallic hydroxides consisting in adding to the bucking liquor, substances which form with the metal compounds soaps that can easily be washed out of the fibres.

4. In a bucking process for vegetable fibrous material, the method of treating the material simultaneously and in one single operation with caustic alkalies and metallic hydroxides, consisting in adding to the bucking liquor a third reagent which prevents the envelopment of the fibres in obstructive metallic soaps and ensures that the final form of the compounds produced with the natural fats and waxes of the fibre during boiling shall be such that substantially all the impurities can be removed from the fibre by simple washing operations.

5. In a bucking process for vegetable fibrous materials the method consisting in boiling the fibrous material to be treated with a liquor containing a caustic alkali and a

metallic salt of a substance adapted to bring the metallic soaps of the fats and waxes in the fibrous material to a state such that the residual matter remaining in the fibre after boiling can be removed by simple washing.

In testimony whereof I affix my signature.

GUSTAV ULLMANN.

**10**

**15**

**20**

**25**

**30**

**35**

**40**

**45**

**50**

**55**

**60**

**65**